

Feb. 27, 1968

E. JOSSO

3,370,940

IRON-NICKEL ALLOYS

Filed Nov. 15, 1966



## 1

3,370,940

**IRON-NICKEL ALLOYS**

Emile Josso, Sauvigny-les-Bois, France, assignor to Societe Metallurgique d'Imphy, Paris, France, a company of France

Filed Nov. 15, 1966, Ser. No. 594,474

Claims priority, application France, Nov. 30, 1965,

40,297

3 Claims. (Cl. 75—122.5)

**ABSTRACT OF THE DISCLOSURE**

Iron-nickel alloys having improved magnetic properties and improved forgeability are obtained by replacing manganese in the alloy by uranium. The nickel content is greater than or equal to 30% and the amount of uranium is from 0.02 to 0.5% by weight.

This invention relates to uranium-containing iron-nickel alloys.

It is well known that vacuum-melted iron-nickel alloys having a nickel content greater than or equal to 30% have excellent magnetic properties. Deoxidised alloys of this kind can be forged and hot-rolled without difficulty if they are prepared from very pure raw materials, but they behave differently if the raw materials used contain sulphur, as is frequently the case with commercial quality materials. The magnetic properties remain substantially unchanged, but the high-temperature deformability deteriorates unless a desulphurising agent is added to the alloy; unless this is done, the product cannot be forged or hot-rolled and despite its good magnetic properties it can be used only for very restricted applications.

To overcome this difficulty, conventional practice is to add a small quantity (for example 0.3—0.5%) of manganese to the melt in order to facilitate forging or hot-rolling of the ingots.

Unfortunately, this addition of manganese, which combines with the sulphur to give a relatively stable sulphide, has an unfavourable effect on the magnetic properties of the alloy, as will be apparent from the following table, which relates to 0.3 mm. thick strip rings originating from three melts prepared under identical conditions with the same raw materials.

## 2

The carbon contents shown in Table I were determined on the ingot prior to any conversion operations. These relatively high contents have the effect of keeping the oxygen concentration of the materials at a very low level of about 10 p.p.m. After rolling into thin strips and after annealing for 6 hours at 1100° C. in purified hydrogen to develop the magnetic properties, this carbon content drops to about 0.01%.

It is well known that uranium has a great affinity for sulphur and oxygen. In steel it forms refractory inclusions of a globular shape which are thought to be oxy-sulphides.

Work on the use of uranium in ferrous alloys has hitherto been devoted to ordinary, alloy or stainless steels solely to improve their mechanical properties. Uranium increases the tensile strength at ambient temperature, increases quenchability and promotes structural hardening. With regard to resistance of stainless steels to corrosion, the results are as yet too incomplete for any definite conclusions to be drawn.

No coherent data is available on the influence of an additional of uranium to binary or complex iron-nickel alloys having a nickel content greater than 30%, such alloys being in widespread use because of their special physical properties (their magnetic, expansion, electrical, mechanical and thermomechanical properties in particular).

Tests have shown the advantage of uranium over magnetic alloys, but uranium was used heretofore only as a deoxidant.

It has been found—and this is one of the features of the invention—that uranium may advantageously completely or partly replace manganese in order that iron-nickel alloys having a nickel content greater than or equal to 30% may be made forgeable.

This improvement of forgeability is obtained by the use of uranium as desulphurising agent and contrary to previous tests it is advantageous to introduce it into material which has previously been satisfactorily deoxidised in order to prevent some of the uranium from being neutralised in the form of an oxide.

It is therefore advantageous for the oxygen concentration not to exceed 100 p.p.m. Processing partially or completely in vacuo or in a protective or reducing gas may be of advantage to give such a low impurity content.

TABLE I

| Reference No.             | Chemical analysis of ingot, percent                                                                                                                                                                                                                                                                                                                                                       | Permeability at 5 milloersteds | Maximum permeability | Coercivity, Oe. |
|---------------------------|-------------------------------------------------------------------------------------------------------------------------------------------------------------------------------------------------------------------------------------------------------------------------------------------------------------------------------------------------------------------------------------------|--------------------------------|----------------------|-----------------|
| 1 (with manganese)....    | {C=0.172, Si=0.02, Mn=0.49.....<br>S=0.0088, P=0.008, Ni=49.09.....<br>O <sub>2</sub> =0.0009, N <sub>2</sub> =0.0011.....<br>(C=0.131, Si=traces, Mn=0.34.....<br>S=0.0089, P=0.005, Ni=49.50.....<br>O <sub>2</sub> =0.0005, N <sub>2</sub> =0.007.....<br>(C=0.122, Si=0.02, Mn=traces.....<br>S=0.0090, P=0.008, Ni=48.98.....<br>O <sub>2</sub> =0.0010, N <sub>2</sub> =0.0019..... | 3,560                          | 39,000               | 0.127           |
| 2 (with manganese)....    | {C=0.131, Si=traces, Mn=0.34.....<br>S=0.0089, P=0.005, Ni=49.50.....<br>O <sub>2</sub> =0.0005, N <sub>2</sub> =0.007.....                                                                                                                                                                                                                                                               | 4,170                          | 39,000               | 0.096           |
| 3 (without manganese).... | {C=0.122, Si=0.02, Mn=traces.....<br>S=0.0090, P=0.008, Ni=48.98.....<br>O <sub>2</sub> =0.0010, N <sub>2</sub> =0.0019.....                                                                                                                                                                                                                                                              | 9,440                          | 78,000               | 0.043           |

A heat treatment was carried out and comprised annealing for 6 hours at a temperature of 1100° C. in hydrogen. The first two melts respectively contained about 0.5 and 0.3% of manganese while the third contained only traces thereof. Although the third melt was unfortunately unforgeable, it had very much better magnetic properties than the first two.

60 This positive effect is clearly demonstrated by the single figure which shows the variation of the deformability (represented in this case by elongation at break) against the test temperature for five iron-nickel alloy ingots containing 48 to 50% of Ni, the compositions of the alloys being given in Table II, the reference numbers of these alloys being shown in the figure.

TABLE II.—CHEMICAL ANALYSES (PERCENTAGES, UNLESS OTHERWISE INDICATED)

| Reference No. | C     | Si               | Mn               | S      | P     | Ni    | O <sub>2</sub><br>(p.p.m.) | N <sub>2</sub><br>(p.p.m.) | Addition |
|---------------|-------|------------------|------------------|--------|-------|-------|----------------------------|----------------------------|----------|
| 3-----        | 0.122 | 0.03             | ( <sup>1</sup> ) | 0.0090 | 0.008 | 48.98 | 10                         | 19                         | None.    |
| 2-----        | 0.131 | ( <sup>1</sup> ) | 0.34             | 0.0089 | 0.005 | 49.50 | 5                          | 7                          | Mn:0.34. |
| 4-----        | 0.036 | ( <sup>1</sup> ) | 0.09             | 0.0078 | 0.005 | 48.98 | 5                          | 6                          | U:0.05.  |
| 5-----        | 0.084 | ( <sup>1</sup> ) | ( <sup>1</sup> ) | 0.0073 | 0.007 | 49.15 | 6                          | 5                          | U:0.10.  |
| 6-----        | 0.110 | ( <sup>1</sup> ) | ( <sup>1</sup> ) | 0.0067 | 0.007 | 49.20 | -----                      | -----                      | U:0.25.  |

<sup>1</sup> Traces.

The deformability of the ingot without a desulphurising addition is practically zero between 500 and 800° C.; above 800° C. it improves, but never reaches a satisfactory level. With an 0.3% manganese addition, the fragility area is reduced but does not completely disappear. Against this, an addition of 0.05 to 0.25% of uranium gives the metal appreciable deformability which in every case is very much greater than that of the alloy containing 0.3% of Mn, as soon as the temperature exceeds 550° C. In practice, this unexpected result means a great improvement in forgeability. Whereas the alloy without an additive is unforgeable, there is no difficulty in forging uranium-containing ingots.

Of course the above-indicated uranium contents are given by way of example and have no limiting force. The

15 Here again the compositions are given by way of example and have no limiting force. The nickel content is preferably between 43 and 55% for the application in question but the superior magnetic quality provided by uranium instead of manganese may be obtained with all ferronickel alloys having a nickel content greater than or equal to 30%. Table IV gives examples of results obtained with melts containing various nickel contents. The 20 corresponding properties were measured on 0.07 mm. thick strip rings annealed for 6 hours at 1100° C. in hydrogen with slow cooling in the furnace in the case of the alloy containing 36% of nickel; in the case of the alloy containing 78% of Ni, the tests were carried out on 0.3 mm. thick strip rings annealed for 6 hours at 1000° C. in hydrogen with rapid cooling from 600° C.

TABLE IV

| Type of alloy                         | S-content by weight Percent | Mn-content by weight Percent | U-content by weight Percent | Permeability at 5 moe. | Maximum permeability | Coercivity, Oersteds |
|---------------------------------------|-----------------------------|------------------------------|-----------------------------|------------------------|----------------------|----------------------|
| Fe-Ni alloy containing 36% of Ni----- | 0.01<br>0.01                | 0.3<br>-----                 | 0.05<br>2,400               | 2,100<br>2,400         | 9,000<br>12,000      | 0.20<br>0.17         |
| Fe-Ni alloy containing 78% of Ni----- | 0.007<br>0.007              | 0.48<br>-----                | 0.06<br>8,900               | 8,000<br>8,900         | 52,000<br>70,000     | 0.09<br>0.065        |

beneficial effect of uranium is found with an addition of as little as 0.02% by weight; with regard to the top uranium concentration limit, this is dictated more by safety requirements in respect of radiation than by technological conditions. The maximum concentration would be limited to 0.5% by weight. Similarly, although Table II and the single figure refer essentially to alloys containing 48–50% Ni, these contents have no limiting force and the beneficial influence of the uranium additive covers all ferronickel alloys having a nickel content greater than or equal to 30%.

It has also been found—and this is another feature of the invention—that for equal forgeability, the uranium additive is much less harmful to the magnetic properties than is the manganese additive. This is clear from Table III, which shows the magnetic properties after annealing for 6 hours at 1100° C. in hydrogen for iron-nickel alloy melts containing 48 to 50% Ni processed under identical conditions and respectively containing 0.34% Mn, 0.05% U, 0.10% U and 0.25% U.

TABLE III

| Reference | Addition    | Magnetic properties              |                      |                 |
|-----------|-------------|----------------------------------|----------------------|-----------------|
|           |             | Permeability at 5 milli-oersteds | Maximum Permeability | Coercivity, Oe. |
| 2-----    | 0.34% Mn--- | 4,170                            | 39,000               | 0.096           |
| 4-----    | 0.05% U---  | 4,830                            | 76,600               | 0.050           |
| 5-----    | 0.10% U---  | 4,370                            | 57,500               | 0.080           |
| 6-----    | 0.25% U---  | 4,680                            | 46,400               | 0.091           |

These properties were measured on 0.3 mm. thick strip rings prepared by conventional industrial techniques and annealed for 6 hours at 1100° C. in purified hydrogen. It will be apparent that magnetic quality decreases as the uranium content increases, but the alloy containing 0.25% of uranium still has a better permeability and a lower coercivity than the alloy containing 0.34% of manganese and it must therefore be considered as being of a superior quality.

40 The main object of the invention is to replace manganese by uranium in magnetic iron-nickel alloys. However, since the improved forgeability provided by uranium is valid irrespective of the use for which the material is intended, the field of application of the invention is not restricted solely to magnetic alloys but relates generally to all binary or complex iron-nickel alloys having a nickel content greater than or equal to 30%, irrespective of 45 use (e.g., magnetic alloys, alloys having a specific expansion, alloys having special elastic or thermoelastic properties, alloys having a specific resistivity, and so on). By complex iron-nickel alloys is meant iron and nickel based alloys which in addition to the impurities inherent in any 50 metallurgical product contain additions of chromium, copper, silicon, molybdenum, aluminum, calcium, or magnesium for example which, without modifying the character or structure of the alloy, contribute towards improving the physical properties thereof.

I claim:

1. Binary iron-nickel alloys, having a nickel content at least equal to 30% by weight, 0.02 to 0.5% by weight of uranium and the remainder iron with the conventional 60 impurities of metallurgical products.
2. Iron-nickel alloys as described in claim 1, containing less than 100 p.p.m. of oxygen.
3. Iron-nickel alloys as described in claim 1, the nickel content by weight being between 43 and 55%.

## References Cited

## UNITED STATES PATENTS

- 70 3,148,978 9/1964 Douglas et al. ----- 75—122.5  
3,221,559 9/1966 Weber ----- 75—122.5 X

CARL D. QUARFORTH, Primary Examiner.

75 M. J. SCOLNICK, Assistant Examiner.